

Feb. 27, 1923.

1,446,947.

T. L. TALIAFERRO.

PROCESS OF DRYING LITHOGRAPHED METAL PLATES.

FILED APR. 7, 1920.



Patented Feb. 27, 1923.

1,446,947

# UNITED STATES PATENT OFFICE.

THOMAS L. TALIAFERRO, OF CHICAGO, ILLINOIS, ASSIGNOR TO PHOENIX HERMETIC COMPANY, OF CHICAGO, ILLINOIS, A CORPORATION OF NEW YORK.

## PROCESS OF DRYING LITHOGRAPHED METAL PLATES.

Application filed April 7, 1920. Serial No. 372,055.

*To all whom it may concern:*

Be it known that I, THOMAS L. TALIAFERRO, a citizen of the United States, residing at Chicago, in the county of Cook, State 5 of Illinois, have invented certain new and useful Improvements in Processes of Drying Lithographed Metal Plates, of which the following is a description, reference being had to the accompanying drawing and to 10 the figures of reference marked thereon.

The invention relates to a new and useful improvement in the process of drying lithographed metal plates, and more particularly to metal plates such as are used in the 15 forming of metal containers, covers, or the like.

An object of the invention is to provide a process of drying lithographed plates, whereby the plate may be quickly dried 20 without any discoloration of the pigments 25 of the lithographing ink.

A further object of the invention is to provide a process whereby the drying of the sheets may be effected during the continuous 25 travel of the sheets.

These and other objects will in part be obvious and will in part be hereinafter more fully described.

The figure of the drawings shows more or 30 less diagrammatically a drying oven for carrying out my improved process.

Prior to my invention, it has been common to decorate metal sheets with ink by various lithographing processes, and then 35 the sheets are dried. This drying of a lithographed sheet has been accomplished by subjecting the sheet to a low heat for a considerable period of time, and this was thought necessary in order to prevent the discoloration 40 of the pigments contained in the ink. It is well known that the drying of a lithograph ink is not a volatilization process, but, on the contrary, is a chemical action, the ingredients oxidizing and thus bringing 45 about a setting or drying of the ink. This oxidation process, which results in the drying of the ink is therefore a progressive or cumulative action, and time is required in order to effect the same. I have discovered 50 that a lithographed sheet of metal may be heated to relatively high temperature so as to increase the rapidity of the chemical action, and the resulting drying of the ink provided that this intense heat to which the 55 ink is subjected, is restricted to a very short

interval of time. The discoloration of the pigments due to heat, is not rapid, but occurs only after the lithograph ink has been subjected to a relatively high temperature for a relatively long period of time. My improved process of drying lithographed plates consists therefore in the heating of the lithographed sheet to a comparatively high temperature so as to bring about a rapid oxidation of the ink and the resulting drying thereof and the restricting of the heating period and the rapid cooling of the sheet after the heating period so as to prevent discoloration of the pigments of the ink. I have found that the sheets may be heated to 60 a temperature from two hundred and fifty degrees to four hundred and fifty degrees and maintained at this temperature for a period of four or five minutes without affecting a discoloration of the pigments provided the sheet is at the end of the heating 65 period withdrawn from the heating chamber and allowed to quickly cool.

Another object of my process consists in the passing of the sheets continuously 80 through a heating chamber wherein the sheet will be quickly raised to the temperature referred to above, and the withdrawing of the sheet from the heating chamber at the end of the period referred to above, and 85 preferably maintaining the sheets in vertical position while they are passing through said heating chamber and for a period of time after they leave the heating chamber. This not only causes the sheet to be quickly heated, to a temperature which brings about the rapid oxidation of the ingredients of the ink, but it also quickly cools the sheet and thus prevents the high temperature effects 90 upon the ink from causing discoloration of 95 the pigments.

In the drawings I have shown one form of apparatus for carrying out the process, and brief reference will be made thereto. The drying oven is indicated at 1 in the 100 drawings and is preferably of the construction described in detail in my Patent #1,318,187, granted October 7, 1919. Passing through the oven is an endless conveyor 2 having vertically extending arms 3 between which the sheets are placed. The endless conveyor is driven in any suitable 105 way and the sheets are fed between the arms by the feeding-in conveyor 4. I have indicated in the drawings the sheets at S. 110

The drying chamber is heated as shown in the drawings by gas burners 5 which are of such a character that the interior of the oven may be maintained at a temperature 5 from two hundred and fifty to four hundred and fifty degrees. At the upper part of the chamber there is a longitudinally extending pipe 6 having openings, and air is supplied to this pipe and allowed to pass into the 10 chamber. The amount of air thus delivered to the chamber is comparatively slight and is mainly for the purpose for causing a movement of the air within the heating oven so as to bring about a uniform distribution 15 of the heat in the oven thus avoiding hot spots and insuring uniform drying of the sheets. At the receiving end of the oven there is a pipe 7 which is provided with openings, and this pipe is connected with a 20 suitable supply of air which causes the blanket of air indicated by the lines 8 to be formed at the entrance of the oven. This blanket of air serves as a door for closing the oven, so as to maintain the heat in the 25 oven. The sheets, however, will readily pass through the blanket. At the delivery end of the oven there is another pipe 9 which forms a blanket of air 10 for closing the delivery end of the oven. Through these air 30 blankets, the oven is substantially closed so that it may be maintained at a relatively high heat between two hundred and fifty and four hundred and fifty degrees throughout the entire extent of the oven. Through 35 this arrangement, the lithographed sheet is subjected to this intense heat just as soon as it enters the oven and the intense heat continues until the sheet passes the blanket at the end of the oven out into the open 40 atmosphere. Through the subjecting of the lithographed sheets to this high temperature, a very rapid oxidation of the ink takes place. The length of the oven and the speed of travel of the conveyor is such that the 45 sheet will be from four to five minutes in passing through the oven, and therefore, the drying process which is brought about through the oxidation of the ingredients of the ink will be substantially effected when 50 the sheet leaves the drying oven. By arranging the sheets vertically the surface of the ink is directly subjected to the circulating heated air in the oven, and is therefore more quickly brought to the maximum 55 temperature of the oven. On the other hand as soon as the sheets pass out of the oven, the vertical arrangement thereof in the open atmosphere brings about a rapid cooling of the metal and the ink, this withdraws the 60 heat from the metal sheet and the ink and prevents the discoloration of the pigments which might result from the heat held in the metal if the metal was not rapidly cooled.

Through the process described above, it 55 will be apparent that I am able to very

quickly bring the lithographed ink to a temperature where the oxidation is very rapid, maintain it for a short interval at this temperature, and then quickly cool the same, and therefore the drying of the sheet is 70 very much more quickly effected, and without any injurious results, such as discoloration of the pigments.

The apparatus which has been described in brief above, forms no part broadly of the 75 present invention, but is described and claimed in my Patent No. 1,399,415, granted Dec. 6, 1921.

I have described the above apparatus for the purpose of making more clear the process. It is obvious that the apparatus for carrying out the process may be widely varied. It is also obvious that the specified temperatures, and the time interval to which the sheet of metal is subjected to 85 the temperature stated, may be varied within suitable ranges. The temperatures and the period of time stated are those preferred. The essential feature of the invention consists however, in the heating of the sheet to 90 a relatively high temperature for producing rapid oxidation of the ingredients of the lithograph ink and restricting the period of heating so as to prevent discoloration of the pigments, and this is greatly aided by 95 the rapid cooling of the sheet after the heating period.

It is obvious that minor changes in the details of construction may be made without departing from the spirit of the invention as set forth in the appended claims. 100

Having thus described the invention, what I claim as new and desire to secure by Letters-Patent, is:—

1. The process of treating lithographed plates consisting in travelling the sheet through a drying oven heated to a relatively high temperature which would, if the operation be continued, carry the oxidization of the ingredients to a point of discoloration of the pigments of the ink, and wherein the air is continuously moving so as to prevent hot spots and to produce a uniform rapid oxidization of the ingredients for drying the ink, and restricting the period of heating so as to stop the oxidization before discoloration of the pigments takes place. 105 110 115

2. The process of drying lithographed plates consisting in travelling the sheets in vertical position through a drying oven heated to a temperature between two hundred and fifty and four hundred and fifty degrees, and wherein the air is continuously moving whereby the rapid uniform oxidization of the ingredients of the ink is brought about, restricting the period of heating to four or five minutes and rapidly cooling at the end thereof so as to prevent discoloration of the pigments of the ink. 120 125

3. The process of drying lithographed 130

- plates consisting in travelling the lithographed sheets in succession through a drying oven heated to a temperature of two hundred and fifty to four hundred and fifty 5 degrees, the speed of travel being such as to subject the sheets to the heat of the oven for a period of between four and five minutes and rapidly cooling the sheet after it leaves the oven.
- 10 4. The process of drying lithographed plates consisting in travelling the lithographed sheets in succession through a drying oven heated to a temperature of two hundred and fifty to four hundred and fifty 15 degrees, the speed of travel being such as to subject the sheets to the heat of the oven for a period of between four and five minutes and rapidly cooling the sheet after it leaves the oven, and closing the receiving and delivering ends of the oven by a blanket of air and causing a circulation of the air within the oven so as to bring about a substantially uniform temperature from one 20 end to the other of the oven.
- 25 5. The process of drying lithographed plates consisting in travelling the sheets in vertical position through a drying oven heated to a temperature between two hundred and fifty and four hundred and fifty degrees, regulating the speed of travel of the sheet so that each sheet will be retained in the oven from a period of four to five minutes, and maintaining the sheets in vertical position in the open air after leaving the oven until the sheets are cooled. 30
6. The process of drying lithographed plates consisting in travelling the sheets in vertical position through a drying oven heated to a temperature between two hundred and fifty and four hundred and fifty 35 degrees, regulating the speed of travel of the sheet so that each sheet will be retained in the oven from a period of four to five minutes and maintaining the sheets in vertical position in the open air after leaving the oven until the sheets are cooled, closing the receiving and delivering ends of the oven by a blanket of air and circulating the air within the oven so as to maintain substantially a uniform temperature from one 40 end to the other thereof. 45

In testimony whereof, I affix my signature.

THOMAS LUCIEN TALIAFERRO.